

June 3, 1930.

L. KIRSCHBRAUN  
ROOFING ELEMENT WITH THICKENED BUTT EDGES  
AND METHOD OF MAKING THE SAME  
Filed July 31, 1926

1,760,873



Fig. 1



Fig. 2



Fig. 3

Fig. 4



Fig. 5



Fig. 6



Fig. 8

Fig. 7

Inventor:

Lester Kirschbraun,  
by  
Kirschbraun and Company  
Attn:

## UNITED STATES PATENT OFFICE

LESTER KIRSCHBRAUN, OF LEONIA, NEW JERSEY, ASSIGNOR, BY MESNE ASSIGNMENTS, TO THE PATENT AND LICENSING CORPORATION, OF BOSTON, MASSACHUSETTS, A CORPORATION OF MASSACHUSETTS

ROOFING ELEMENT WITH THICKENED BUTT EDGES AND METHOD OF MAKING THE SAME

Application filed July 31, 1926. Serial No. 126,279.

This invention relates to fabricated roofing elements and has special reference to elements formed with a relatively narrow bead or line of extra thickness adjacent to the butt edge thereof.

Roofing of the type referred to is customarily made of felted fibrous sheet material composed of rag or asbestos fiber or the like, felted together on a paper-making machine.

- 10 This fibrous sheet material is somewhat loose and porous in structure so as to be capable of taking up a considerable quantity of liquid saturant. Suitable waterproofing material, such as low melting-point asphalt, pitch or 15 the like, is used to impregnate the fibrous sheet, after which it is coated with high melting-point asphalt to provide an impervious protecting layer which will be thoroughly waterproof and will not run or flow 20 under the heat of the sun when laid on the roof. The asphalt coating where exposed to the weather is usually protected by a layer of mineral granular material such as crushed slate, tile, brick, or the like, which is applied 25 to the asphalt coating while the latter is still hot and sticky. Enough of the granular material is pressed into and partially embedded in the asphalt coating to cover the same completely and to protect it from the 30 direct action of the weather. From sheet material thus prepared by impregnating, coating and slating, as described, individual roofing elements of any desired shape and size are cut. Elements so prepared, however, 35 are of relatively thin unsubstantial appearance when laid on a roof, and it has been found that if the butt edges, which are the most conspicuous part of the laid element to the observer, are suitably thickened, the 40 result is a very marked improvement in the general appearance of the roof. The thickening of the butt edge portions of the element also serves to stiffen the exposed portions of the shingle and to prevent warping and curling of the corners of shingle-simulating tabs which are found in many of the more popular 45 types of strip shingles. Roofing elements cut from a sheet of prepared roofing, as described, are also subject to a serious defect due to the 50 cut edges which result from the operation of cutting the sheet into the individual elements. These cut edges leave cut ends of fibers exposed to the weather along the butt edge of the roofing element when laid and provide a means for the absorption of atmospheric moisture by the fibers of the felt base of the roofing element. The absorption of moisture into the roofing element in this way and the evaporation of moisture therefrom in dry weather, together with other effects of 55 the weather, result in a tendency on the part of the felt base to "sponge" and of the exposed portions of the roofing element to warp and curl, thus reducing the weather-proofing quality of the roof as a whole and 60 shortening the life of the individual elements. Thus in applying material to the edge portion of a roofing element to thicken the same, it is advantageous to coat the butt edge itself as well as the edges of the slots which may 65 have been cut in the element to define shingle-simulating tabs. By my invention, I provide a method for accomplishing these desirable results, that is, for sealing the cut edges of the element which are to be exposed to the 70 weather and positively forming a bead on the under side of the portions adjacent to the cut edges which will both stiffen these edges and add materially to the appearance of the roof as a whole when laid.

The invention can be better understood by reference to the drawing, of which:—

Figure 1 is a diagrammatic elevation of one form of apparatus for applying a coating of asphalt to the exposed surface and edges of a 85 strip shingle in such a way that a narrow bead will be formed on the reverse side adjacent to the butt edge.

Figure 2 is an end elevation of the same.

Figure 3 is a view of a plurality of strip shingles so treated, showing their appearance when laid on a roof.

Figure 4 is a view of the under side of a strip shingle of slightly different shape showing the disposition of the beading along the 95 cut edges of the butt portion.

Figure 5 is an elevation of another form of apparatus for applying asphalt to one face and the butt edges of a strip shingle.

Figure 6 is an end elevation of the same.

100

Figure 7 is a vertical section of a strip shingle which has been coated on its exposed surface and edges and has been provided with a bead on the portion adjacent the butt edge.

5 Figure 8 is a diagrammatic view of another apparatus for coating and beading roofing elements.

Referring to the drawings in detail, Figures 1 and 2 show a spout or nozzle 10 which 10 is suitably shaped to supply a vertically elongated jet of molten asphalt against the butt portion of the upper face of a strip shingle 11 which is suspended vertically as by suitable clamps 12 and conveyed in an endwise 15 direction past the spout 10. The strip 11 may be a saturated felt blank cut to shape, or it may be a roofing element cut from a sheet of coated and slated roofing such as is frequently put on the market as a finished product. Beneath the path of the strip shingle 20 11 is located a member 13 having a channel 14 formed in the top thereof and extending in the direction of motion of the strip shingle. The member 13 is so arranged that the butt 25 edge portion of the strip shingle will travel therein as the shingle is progressed. Excess asphalt from the spout 10 will flow down into the channel 14 and keep it filled so that the asphalt therein will adhere to the reverse 30 or under face of the strip shingle adjacent to the butt edge and will thus form a bead thereon beside coating the butt edge itself. The designation of the faces of the shingle as "upper" and "under" has reference to the 35 shingle as laid on a roof. It is obvious that the jet from the spout 10 will project through the cut-outs 15 of the strip, whatever shape these cut-outs may be, and will coat the cut edges thereof so that in this way the exposed portion of the upper face and the exposed 40 cut edges will all be completely coated with a continuous layer of asphalt and a bead will be formed on the portion of the under face of the shingle adjacent to the butt 45 edge. If the strips which are being coated are formed with rectangular tabs having vertical side edges (as that shown in Figure 5), some of the asphalt which is projected through the slots in the strip will creep 50 around the edges to the rear face as it trickles down and will form beads adjacent to these edges on the rear face of the strip. In order to maintain the asphalt which collects in the channel 14 in fluid condition, the member 13 55 may be kept heated as by a steam pipe 16 or other suitable means. The spout may be adjusted vertically to regulate the upper limit of the coating applied thereby on the face of the shingle strip. If the latter has 60 been cut from a coated and slated sheet, it is preferable to put the additional face coating only on the exposed portion of the face, that is, to such a height on the strip that the upper limit of the extra coating will 65 be approximately in line with the butt edges.

of the strips in the course laid next above on thereof. In the case of certain shapes of strips, as for example that shown in Figure 3, small portions of the strip will appear through the cut-outs above the butt-edge line 70 of the course above. By surfacing the extra coating with slate or grit of a color different from that used in surfacing the sheet from which the strip was cut, artistic effects may be produced in the pattern of the roof when 75 laid.

Figures 5 and 6 illustrate a modified form of apparatus for accomplishing the same result. In this case, the shingle strip 11 is vertically suspended as by clamps 12 and is 80 carried along edgewise past a suitable spout 10. Instead of a channeled block for receiving the butt edge of the shingle, I provide in this case a series of pairs of rolls 17, 18 supported over a suitable container in angular 85 relation to each other. The strip shingle 11 is preferably supported in such a way that its butt edge rides on the rollers 17 while a narrow portion of the reverse side of the strip adjacent the butt edge contacts with 90 the rollers 18. The rollers 18 are preferably mounted for adjustment transversely of the container 19, this adjustment being for the purpose of regulating the width of the bead 95 of asphalt applied to the rear face adjacent to the butt edge. The asphalt from the nozzle 10 is directed against a portion of the surface of the strip shingle, the excess asphalt flowing downwardly and being distributed over the rollers 17, 18 or being caught 100 by the container 19 beneath. The rollers may be kept heated to prevent the congealing of asphalt thereon by any suitable means. This can be easily accomplished by arranging them to be partially immersed in the hot 105 asphalt held by the container 19, the latter being supplied with steam pipes or equivalent heating means. This apparatus produces the same result as that shown in Figures 1 and 2, namely, a coating on the exposed 110 portion of the front face of the strip shingle, on the exposed cut edges, and on the portion adjacent to the butt edges.

Another form of apparatus is illustrated in Figure 8. This comprises essentially a series 115 of clamps 20 carried by a conveyor 21 and adapted to support strip shingles 11 vertically for motion in a direction perpendicular to their planes. In the path of the strip shingle is located a coating roll 22 which may dip directly into a supply of molten asphalt in a container 23 or may be fed therefrom as by a feed roll 24. The rolls 22 and 24 are preferably geared together and are positively driven by suitable driving connections 120 (not shown). Where coating asphalt is applied to strip shingles by a roll as in this case, it is desirable to pre-heat the shingles to insure a firm adhesion of the coating thereto. This may be done by any desired means such 125 130

as an oven, through which the shingle may be carried by the conveyor. As each shingle strip is brought into contact with the coating roll 22, it is allowed to swing to a tilted position as it is dragged over the surface of the roll, the clamps 20 being swingably mounted to allow free tilting motion of the strip shingles. The roll 22 is preferably driven in the direction of the conveyor at a peripheral speed somewhat greater than the linear speed of the conveyor 21, this resulting in a heaping up of coating material, as at 25, against the edges of the butt and cut-outs as the shingle rides over the uppermost portion of the roll 22. The heaped up asphalt flows over the portions of the rear face of the shingle adjacent to the butt edges and the edges along the cut-outs, thus forming a bead 26 on those portions as indicated in Figure 7. It is to be understood that the element or shingle 11 shown in this figure may have been cut from a sheet of finished roofing material, i. e., roofing felt which has been saturated, coated and slated in a manner well known in the art. The various layers of material making up the sheet from which the element 11 is cut are not indicated in Figure 7, the object being to avoid confusion of detail. This results in a face coating 27 of asphalt on the forward face of the strip shingle and also in a thorough coating all over the cut edges of the butt and cut-out portions.

It will be noted that this form of apparatus is capable of coating any desired amount of the exposed face of the roofing element and also of forming a bead on the reverse face not only along the lower butt edge, but also along the edges of the cut-outs regardless of the shape of the latter. In the form of strip shingle shown in Figure 4, for example, the forms of apparatus illustrated in Figures 1 and 5 would not be capable of forming the complete bead 26 adjacent to all the edges of the butt portion and cut-outs of the shingle, but would simply coat the front face and the edges themselves. In the case of a shingle strip formed with rectangular tabs as illustrated in Figure 5, however, the apparatus shown in Figure 5 will not only positively deposit a bead along the butt edge of the shingle, but a bead will also be formed part way up the side edges of the cut-outs by some of the asphalt which is projected through the slots from a spout 10 and creeps around the vertical edges of the cut-outs.

The face coating 27, the edge coating and the bead 26 are preferably surfaced with comminuted material, such as crushed slate or the like, to protect the coating from the action of the weather. The surfacing material is applied while the asphalt is hot and sticky and is pressed into the asphalt so that the particles are partially embedded therein and are firmly held in place. The surfacing step,

as well as the application of the asphalt, may be performed by hand, or suitable mechanism may be provided for that purpose.

I am aware that strip shingles have heretofore been formed by applying a sealing coat over the exposed areas of the front face and over a corresponding area of the rear face as well as the cut edges. The strip shingle produced by my invention as described hereinbefore has the advantage of lighter weight, while affording the same appearance of thickness on the roof and the same amount of protection. The tabs also tend to lie closely against the course below since the weight of the tabs rests upon the narrow beads adjacent the butt edges. Roofing elements of this type also effect a considerable saving in coating asphalt without reducing the protective qualities of the shingle. It is obvious that this invention can be applied to roofing elements of the single or multiple type of practically any shape, a few forms of the strip shingle type being illustrated in the drawing by way of example.

I am aware also that strip shingles have been recoated on a face of their butt portions in such a way that the coating material has been allowed to run over the cut edges of the butt portion and to work under the edges to some extent. Such effects heretofore have been purely adventitious and no means have been disclosed for insuring the formation of a continuous bead along the portions of the back face of the element adjacent to all the edges of the butt and cut-outs. By my invention, I provide such means for positively extending the extra coating on the front face to form a bead on the back face adjacent to the edges, thereby giving the maximum thickness at the butt edge.

Having thus described an embodiment of my invention, it should be evident to those skilled in the art that many changes and modifications may be made therein without departing from its spirit or scope as defined by the appended claims.

I claim:

1. Steps in the manufacture of roofing elements, which comprise applying a waterproofing coat to the exposed portion of the upper face of a roofing element, and extending said coat to cover the exposed edges of the element and to form a narrow marginal area of coating on the under face thereof adjacent the butt edges.

2. Steps in the manufacture of roofing elements, which comprise applying a coating of waterproofing material to the exposed portion of the upper face of a roofing element, extending said coating to cover all exposed edges of the element and to form a narrow marginal area of coating on the under face of the element adjacent to the butt edges, and surfacing said coating with grit.

3. Steps in the manufacture of roofing ele-

70

75

80

85

90

95

100

105

110

115

120

125

130

- ments, which comprise applying a coating of waterproofing material to the exposed portion of the upper face of a roofing element, extending said coating to cover all exposed edges of the element and to form a narrow marginal area of coating on the under face of the element extending continuously along all said edges and adjacent thereto, and surfacing said coating with grit.
10. 4. A roofing element having a coating of waterproofing material covering the exposed portion of the upper face of the element and the adjacent edges of the element and forming a continuous narrow marginal area of coating on the under face of the element adjacent to said edges, and a surfacing of grit adhering to said coating.
5. Steps in the manufacture of strip shingles having slots extending upwardly from their butt edges, comprising applying a coat of waterproofing material to the exposed portion of the upper face of a strip shingle, and extending the coating material over all the edges of said exposed portion, including the butt edges, the edges of the slots, and the exposed end edges, and forming with said coating a narrow marginal layer extending on the under face of the shingle continuously along and adjacent to all said coated edges.
20. 6. A strip shingle with slots extending upwardly from the butt edge thereof to define tabs, said shingle having a coating of waterproofing material covering the exposed portion of the upper face thereof and extending over all the edges bounding said exposed portion, said coating also forming a narrow marginal layer on the under face of the shingle extending continuously along and adjacent to the coated edges.
25. 7. Steps in the manufacture of a roofing element, which comprise forming a film of molten coating material, bringing one face of a cut-out roofing unit in contact with said film and heaping coating material along the butt edges of the unit and upon the opposite face of the unit along the butt edges thereof.
30. 8. Steps in the manufacture of a roofing element, which comprise forming a film of molten coating material, bringing one face of a cut-out roofing unit in contact with said film and causing said film to move relatively to said unit in a direction from the butt edge of the unit toward the head thereof, whereby a portion of said film is heaped against the butt edges of the unit and on marginal portions of the unit adjacent to the butt edges.
35. In testimony whereof I have affixed my signature.

LESTER KIRSCHBRAUN.